

## UNITED STATES PATENT OFFICE

KARL BORMANN, OF LEVERKUSEN-ON-THE-RHINE, GERMANY, ASSIGNOR TO GENERAL ANILINE WORKS, INC., OF NEW YORK, N. Y., A CORPORATION OF DELAWARE

## UNIFORM DYEING OF VISCOSE

No Drawing. Application filed February 9, 1929, Serial No. 338,891, and in Germany February 17, 1928.

The present invention relates to the uniform dyeing of viscose silk of different origin.

It is known that it is very difficult to obtain even shades in the dyeing of viscose of different origin, for example of knitted artificial silk.

According to the present invention these difficulties are overcome by dyeing viscose with azo dyestuffs of the general formula:



wherein  $R'$  stands for the residue of any coupling component and  $R''$  stands for a benzene nucleus which may be substituted by 15 a sulphonic or carboxylic acid group, to which the azo group is attached in meta or para position to  $x$ , and  $x$  stands for an azo or azoxy group.

The dyestuffs used for the purpose of my 20 invention are obtainable by the combination of tetrazo compounds of m- and p-azoxylaniline and substitution products thereof with any desired coupling components, or by coupling the diazo compounds of 3- and 4-nitro- 25 aniline or substitution products thereof with any desired component and subsequent reduction of the resulting monoazo dyestuffs with alkaline reducing agents, for example, grape sugar in alkaline solution, to the disazo-azoxy 30 dyestuffs or trisazo dyestuffs.

The dyeing is carried out in the usual manner as outlined in the examples, by dissolving the dyestuffs in hot water and adding to the dye-bath Glauber's salt and monopol soap (a 35 water soluble salt of sulfonated castor oil), if desired with the addition of a wetting agent, f. i. an alkyl-naphthalene-sulfonic acid, such as isobutyl-naphthalene-disulfonic acid. The viscose is introduced into the bath at 40 about 30° C., then the bath is slowly heated

The invention is illustrated by the following examples, without being limited thereto:

Example 1.—10 kgs. of knitted viscose are dyed in 300 liters of water. To the dye-bath are added 200 gms. of the dyestuff, obtained by coupling the diazo compound of 4-nitraniline-2-sulfonic acid with 2-naphthylamine-7-sulfonic acid and linking two molecules of the resulting monoazo dyestuff by treatment with alkaline reducing agents. 200 gms. of 55 monopol soap (a water soluble salt of sulfonated castor oil) and 2 kgs. of Glauber's salt are added. Dyeing is effected for one hour at about 80° C. and is followed by rinsing and drying. The fabric is dyed uniformly a reddish blue shade.

Example 2.—The dye-bath is prepared with 200 gms. of the dyestuff, obtained by coupling the diazo compound of 3-nitraniline with 2-naphthol-8-monosulfonic acid and 70 linking two molecules of the resulting monoazo dyestuff by treatment with alkaline reducing agents, in 300 liters of water. 10 kgs. of knitted viscose are introduced into the dye-bath, which is then heated, 200 gms. of 75 monopol soap and 2 kgs. of Glauber's salt are added, and the dyeing is completed within an hour at about 80° C. The fabric is dyed a uniform orange.

Example 3.—10 kgs. of knitted viscose are 80 dyed in 300 liters of water. To the dye-bath are added 200 gms. of the dyestuff, obtained by coupling the diazo compound of 4-nitraniline-2-sulfonic acid with phenol, methylating 85 the hydroxy group of the monoazo dyestuff and linking two molecules of the resulting monoazo dyestuff by treatment with grape sugar in alkaline solution to the corresponding disazo-azoxy dyestuff, having probable 90 the formula:



45 to about 80° C., at which temperature the viscose is dyed for about 3/4 to 1 hour. Then the viscose is washed and dried.

The dyeings thus obtained are distinguished by their uniformity.

200 gms. of monopol soap and 2 kgs. of Glauber's salt are added. Dyeing is effected for one hour at about 80° C. and is followed by rinsing and drying. The fabric is dyed uniformly a gold orange shade.

Further examples giving the shades obtainable from the various dyestuffs are compiled in the following table:

| Disazoazoxy compound or trisazo dyestuff from the monoazo dyestuff |                                                                                                | Dyes uniformly  |
|--------------------------------------------------------------------|------------------------------------------------------------------------------------------------|-----------------|
| 5                                                                  | 4 - nitraniline - 2 - sulfonic acid + 1 - naphthyl - amine - 4 - sulfonic acid.                | Reddish blue    |
|                                                                    | 4 - nitraniline - 2 - sulfonic acid + 2 - naphthyl - amine - 6 - sulfonic acid.                | Reddish blue    |
|                                                                    | 4 - nitraniline - 2 - sulfonic acid + 1 - naphthol-4-sulfonic acid.                            | Bordeaux        |
|                                                                    | 4 - nitraniline - 2 - sulfonic acid + 2 - naphthol-7-sulfonic acid.                            | Wine red        |
| 10                                                                 | 4 - nitraniline - 2 - sulfonic acid + 2 - methylamino - naphthaline - 7 - sulfonic acid.       | Blue            |
|                                                                    | 4 - nitraniline + 2 - naphthol - 3 : 7 - disulfonic acid.                                      | Reddish blue    |
|                                                                    | 4 - nitraniline + 2 - naphthol - 6 : 8 - disulfonic acid.                                      | Violet          |
| 15                                                                 | 4 - nitraniline + 2 - naphthol - 8 - mono-sulfonic acid.                                       | Wine red        |
|                                                                    | 3 - nitraniline + 1 - naphthylamine - 4,7-disulfonic acid.                                     | Orange          |
|                                                                    | 6 - nitraniline + 1 - naphthol - 3,6 - di-sulfonic acid.                                       | Reddish orange. |
|                                                                    | 4 - nitraniline - 2 - sulfonic acid + pyrazolone from dehydrothiotauidine-monosulfonic acid.   | Orange          |
| 20                                                                 | 4 - nitraniline - 2 - carboxylic acid + pyrazolone from dehydrothiotauidine-monosulfonic acid. | Orange          |
|                                                                    | 4 - nitraniline + 1,8 - dihydroxy - naphthaline - 4 - sulfonic acid.                           | Violet          |
|                                                                    | 4 - nitraniline + 2,5 - aminonaphthol - 1,7 - disulfonic acid.                                 | Bordeaux        |
| 25                                                                 | 4 - nitraniline - 2 - sulfonic acid + 2,5 - aminonaphthol - 7 - sulfonic acid (acid coupling). | Blue            |
|                                                                    | 4 - nitraniline + 2,8 - aminonaphthol - 3,6 - disulfonic acid (acid coupling).                 | Blue            |

4. As new products of manufacture knitted viscose dyed with a dyestuff as claimed in claim 1.

5. As new products of manufacture knitted viscose dyed with a dyestuff as claimed in claim 2.

6. As new products of manufacture knitted viscose dyed with the dyestuff claimed in claim 3.

In testimony whereof I have hereunto set my hand.

KARL BORMANN. [L.S.]

I claim:

1. The process for the uniform dyeing of viscose of various origin, which comprises dyeing the viscose in the customary manner with a dyestuff of the general formula:



25 wherein  $R'$  stands for the residue of any coupling component,  $R''$  stands for a benzene nucleus which may be substituted by a sulfonic or carboxylic acid group and which benzene nucleus is attached to the azo group in one of the positions consisting of the para and meta positions to  $\alpha$ , and  $\alpha$  stands for one of the groupings consisting of the azo- and azoxy-groups.

40 2. The process for the uniform dyeing of viscose of various origin, which comprises dyeing the viscose in the customary manner with a dyestuff of the general formula:



50 wherein  $R'$  stands for the residue of any coupling component,  $R''$  stands for a benzene nucleus which may be substituted by a sulfonic or carboxylic acid group and which benzene nucleus is attached to the azo group in one of the positions consisting of the para- and meta positions to the azoxy group.

55 3. The process for the uniform dyeing of viscose of various origin, which comprises dyeing the viscose in the customary manner with a dyestuff of the formula:



70

75

70

75

80

85

90

95

100

105

110

115

120

125

130